

June 20, 1944.

S. L. BURGWIN

2,351,922

TREATMENT OF SILICON-IRON ALLOYS

Filed March 28, 1941

2 Sheets-Sheet 1

Fig. 1.



Fig. 2.



Fig. 3.



WITNESSES:

J. J. Welles.  
D. C. Gonneau

INVENTOR  
Stephen L. Burgwin.

BY  
James J. Ely  
ATTORNEY

June 20, 1944.

S. L. BURGWIN

2,351,922

TREATMENT OF SILICON-IRON ALLOYS

Filed March 28, 1941

2 Sheets-Sheet 2

Fig. 5.



Fig. 4.



WITNESSES:

J. J. Miller  
R. C. Groome

Fig. 6.



Fig. 7.



INVENTOR

Stephen L. Burgwin.

BY

James P. Ely  
ATTORNEY

## UNITED STATES PATENT OFFICE

2,351,922

## TREATMENT OF SILICON-IRON ALLOYS

Stephen L. Burgwin, Wilkinsburg, Pa., assignor to Westinghouse Electric & Manufacturing Company, East Pittsburgh, Pa., a corporation of Pennsylvania

Application March 28, 1941, Serial No. 385,759

8 Claims. (Cl. 148—21.5)

This invention relates generally to magnetic material and to the heat treatment of silicon-iron alloys to reduce magnetostriction.

Silicon-iron alloys containing up to 6% of silicon have been utilized for a number of years as the magnetic material in different electrical apparatus, and particularly as the core member of transformers. Many processes and methods have been employed for heat treating the silicon-iron alloys and fabricating them into sheet or strip form suitable for use as the magnetic cores of electrical apparatus. The known processes and methods have for their objective the development of the magnetic characteristics of the alloys by reducing the impurities in the alloys, relieving working strains, and/or imparting a preferred orientation to the grain structure of the alloy. The silicon-iron alloys now commercially produced in sheet or strip form have excellent magnetic characteristics.

In a number of commercial installations of electrical apparatus, such as large power transformers, which utilize the now commercially produced silicon-iron alloys in strip form as the magnetic core member, it has been found that undesirable and objectionable noise is developed when the transformer is energized. The noise developed in a transformer can be traced directly to the magnetostriction of the silicon-iron alloy sheets or strips utilized as the core member of the transformer. The magnetostriction of magnetic material is recognized as being the expansion and contraction of the magnetic material when subjected to a magnetizing force. For the purpose of this invention, the kind of magnetostriction of particular interest and the quantity to be measured is  $\Delta L/L$  or the change in length per unit length in the direction of magnetization under the magnetizing force applied.

An object of this invention is to provide for reducing the magnetostriction of silicon-iron alloys which have been fabricated into strip form and treated to develop the magnetic characteristics of the alloy.

A more specific object of this invention is to subject silicon-iron alloys which have been fabricated into strip form and treated to develop the magnetic characteristics of the alloys to an annealing treatment under tension to effectively reduce the magnetostriction of the alloy strip.

Other objects of this invention will become apparent from the following description when taken in conjunction with the accompanying drawings, in which:

Figure 1 is a schematic representation of the

apparatus employed in practicing the method of this invention,

Fig. 2 is a schematic plan of test apparatus utilized in measuring the magnetostriction of alloy strips produced in accordance with this invention,

Fig. 3 is a view in elevation, with a part removed, of a portion of the apparatus of Fig. 2,

Fig. 4 is a graph, the curves of which illustrate the magnetostriction values obtained on alloy strips by utilizing the test apparatus of Fig. 2,

Fig. 5 is a schematic plan of a further test apparatus utilized for measuring the magnetostriction of assembled core members such as are employed in transformers,

Fig. 6 is a graph, the curves of which illustrate the losses encountered in alloy strips treated in accordance with this invention as compared with the losses found in similar alloy strips which have been subjected to only a part of the treatment of this invention, and

Fig. 7 is a graph illustrating the magnetostriction as measured by the apparatus of Fig. 5 for core members of transformers which have been given different treatments.

The silicon-iron alloys containing up to 6% of silicon are well known and the processes for developing the magnetic characteristics of such alloys have been commercially practiced in the past. For example, silicon-iron alloys containing up to about 4½% of silicon are commercially produced in sheet or strip form by subjecting them to different heat treatments, including the step of cold rolling them to the final stages and then subjecting the resulting strip to an anneal at a temperature of 900° C. or higher to develop the magnetic characteristics of the alloys. Silicon-iron alloys containing higher contents of silicon up to about 6% are not being commercially produced by cold rolling processes, since the higher silicon content renders them somewhat brittle and it has therefore become customary to hot work such alloys to the final stages after which a final anneal is employed for relieving working strains. Other methods are well known and practiced for developing the magnetic characteristics of the silicon-iron alloys containing up to 6% of silicon.

In order to reduce the magnetostriction of the commercially produced silicon-iron alloys containing up to 6% of silicon, in accordance with this invention the commercially produced alloy sheets or strips are subjected to a further heat treatment whereby the alloyed components of the strip are in such a condition that the mag-

netostriction of the commercially produced alloys is effectively reduced. For the purposes of this invention the terms sheet and strip are synonymous in their meaning as employed in this application.

Referring to Fig. 1 of the drawings, there is schematically illustrated a representative apparatus for practicing the method of this invention. The apparatus consists of an annealing furnace 10 having open ends through which the strip 12 of silicon-iron alloy which has already been treated and fabricated to develop its magnetic characteristics is passed from a supply reel 14 to a winding reel 16. A brake 18 is associated with a supply reel 14 for applying a suitable drag thereto to impart a predetermined tension to the sheet or strip 12 as it is drawn through the annealing furnace 10, the purpose of which will be explained more fully hereinafter. The open ended furnace 10 can be heated by any suitable means (not shown) for developing the required heat to which it is desired to subject the strip 12 as it passes through the furnace.

In giving the sheet or strip 12 of silicon-iron alloy the treatment of this invention, it is found desirable to heat the strip to a temperature above the Curie point and below 825° C. A preferred range for heating the strip 12 is at a temperature between 700° C. and 825° C. The tension applied to the strip 12 as it is subjected to the annealing temperature is below the elastic limit of the alloy strip and preferably between 500 and 2000 pounds per square inch. The elastic limit as employed in describing this invention and in the claims is a point on the stress-strain curve which represents a stress equal to half of the maximum stress which the strip will bear at the heating temperature without breaking. Where tension below the elastic limit defined hereinbefore is applied for short periods of time such as one to two minutes, it is found that no permanent elongation, except that which is concomitant by the tensioning within the elastic limit, results. In practice the strip 12 is drawn through the furnace 10 at a speed which will permit the heating of the strip to the desired annealing temperature while the winding reel 16 is positioned far enough away from the furnace 10 to permit the strip 12 to cool to a temperature of about 100° C. before it is wound on the reel 16.

It is not known exactly what change takes place in the components or structure of the alloy when subjected to the hereinbefore described annealing treatment under tension. The results obtained, however, illustrate quite definitely that the tension applied during the anneal in air at a temperature between the Curie point of the alloys and 825° C. cooperates to effectively reduce the magnetostriction of the commercially produced silicon-iron alloy strip.

In order to illustrate the beneficial effects of the treatment of this invention, reference may be had to Fig. 4 of the drawings, the curves of which illustrate the magnetostriction of silicon-iron alloy sheets or strips after different treatments. Curve 20 represents a measure of magnetostriction for a silicon-iron alloy strip which contains about 3½% silicon as measured at different flux densities in a strip having surfaces which are free from films. Curve 22 represents the measure of magnetostriction for a strip of the same material when subjected to only the heat treatment utilized in the method of this invention. Curve 24 represents the magnetostriction of another strip of the same material

which has been subjected to the annealing treatment of this invention under tension.

In particular, curve 22 represents the measure of magnetostriction obtained by subjecting the commercially produced silicon-iron alloy sheet or strip to a temperature of 700° C. in air while curve 24 represents the measure of the magnetostriction obtained for the same commercially produced silicon-iron alloy strip when subjected to an annealing temperature of 700° C. while maintained under a tension of 2000 pounds per square inch. From the curves it is quite evident that the treatment of this invention effectively reduces the magnetostriction of the commercially produced silicon-iron alloy strip.

Since the methods of measuring magnetostriction are not well known, and since it has been found necessary to utilize more than one method for measuring the magnetostriction, it is believed to be desirable to briefly explain the apparatus and method employed in measuring the magnetostriction as represented by the curves 20, 22 and 24 of Fig. 4 of the drawings.

Referring to Fig. 2 of the drawings, there is illustrated the apparatus for measuring the magnetostriction of silicon-iron strips employing a direct current excitation means. In this apparatus the magnetic circuit consists of four strips 26 of the silicon-iron alloy arranged with double lap joints in a 25 cm. test frame. The magnetostriction of only one of the strips 26 is measured, the other three strips serving to complete the magnetic circuit. The test strip 26 whose magnetostriction is to be measured is clamped as by means of the screws 28 in a non-magnetic holder formed of the two bars 30 and 32, the holder being disposed to slide over the strip 26. The bar 32 carries bronze bearing balls 34, as shown in Fig. 3, upon which the test strip 26 rests.

In order to measure the elongation of the test strip 26, a roller member 36 having a mirror 38 at one end thereof is disposed between the test strip 26 and the bar 30 of the holder for rotating when the test strip 26 is elongated. As illustrated, the mirror 38 is so positioned as to deflect a beam of light from a lamp 49 which is focused upon a split photox unit 42 which is disposed to be connected to a galvanometer 44 by means of the switch 46, so that the deflection of the galvanometer is proportional to the deflection of the light beam upon the photox unit.

In order to energize the magnetic circuit formed by the strips 26, a source of direct current, such as the battery 48, is disposed to be connected through the double-throw switch 50 to the winding 52 disposed about the strips forming the core member. Variable resistors 51 and 53 are connected in series with each other and the battery, a switch 55 being provided for shunting resistor 53. The double-throw switch 50 is employed for controlling the direction of the energization of the assembled test specimen.

Since it is desired to measure both the elongation of the test strip 26 and the flux densities under which such elongation is obtained, a winding 54 is disposed about the assembled test strips 26 and is adapted to be connected to the galvanometer 44 by means of the double-throw switch 46. Thus with the rotation of the mirror 38 deflecting the light beam on the photox unit 42, a measure of the elongation of the strip 26 can be obtained on the galvanometer 44 as well as a measure of the flux density causing the measured elongation.

Another winding 56 is disposed about the test

strip 26 whose elongation is being measured and the opposite test strip 26 of the core and is connected to a battery 58 for compensating for the earth's magnetic field whereby symmetrical magnetostriction measurements for magnetization of the test strip 26 in both directions may be obtained. The apparatus illustrated in Figs. 2 and 3 is found to give consistent results for magnetostriction for inductions up to 20,000 Gausses.

In operation with the apparatus and test sheet or strip 26 set up as shown in Figs. 2 and 3, the double-throw switch 46 is thrown to the right to connect winding 54 to the galvanometer 44. The double-throw switch 50 is then moved to the right to connect the battery 48 to winding 52 to energize it. Resistor 51 is then adjusted until the induction as measured by the galvanometer upon reversal of switch 50 is equal to the desired value at which the test is to be conducted. Resistor 53 is then adjusted to a value where the simultaneous reversal of the double-throw switch 50 and the opening of switch 55 so affects deenergization of winding 52 that the galvanometer 44 indicates zero induction. With this adjustment of the resistors 51 and 53, when the switch 46 is thrown to the left to connect the photox unit 42 in circuit with the galvanometer 44, the deflection of the galvanometer which occurs upon the simultaneous reversal of switch 50 and the opening of switch 55, is a measure of the magnetostriction of the strip 26 under test. That this deflection is a measure of the magnetostriction is quite apparent in that the roller 36 and mirror 38 move as the test strip contracts as the induction is changed from the maximum desired value to zero induction by operating the switches 50 and 55. This measure of magnetostriction is for a unit length of the test strip extending from the center line of the overlapping joint at the secured end of the test strip to the point of contact of the roller 36.

In order to illustrate that the method of this invention is effective for reducing the magnetostriction of the silicon-iron alloy sheets or strips when built into a core member of a transformer, a different method had to be devised for measuring the magnetostriction of the assembled core member.

Referring to Fig. 5 of the drawings, there is shown the apparatus utilized for measuring the magnetostriction of a core member 88. In this apparatus the core member 88 is built up on a support 90 of non-magnetic steel and is clamped in position by means of a top clamping frame (not shown) secured to the support 90. A winding 92 is provided about the core member 88 and disposed to be connected to a 60-cycle source of power. Matched vibration pick-ups 94 are positioned at each end of one of the legs of the core member 88 and are electrically connected in series to an amplifier 96 which, in turn, is electrically connected to a wave analyzer 98. The core member is then energized at different flux densities at 60-cycle excitation and the vibrations of the leg of the core member measured to obtain the magnetostriction effect of the core member.

The vibration pick-ups 94 are well known and need not be described or shown in detail, the pick-ups consisting generally of a small coil floating in a magnetic field produced by a permanent magnet firmly attached to the case of the pick-up with a rod extending from the case of the pick-up to the vibrating member whereby the casing of the pick-up will vibrate while the

coil, due to its inertia, will tend to remain substantially fixed.

With the pick-ups 94 disposed at the opposite ends of a leg of the core member 88 as shown in Fig. 4, and connected in series opposition, the vibrations for given inductions are recorded through the amplifier and the wave analyzer. The pick-ups are disposed at a number of different locations at the end of the leg of the core member in order to get an average recording of the vibration of the core member. In recording the vibrations, the amplitude of the 120-cycle fundamental frequency alone is measured since for the purpose of this invention it is very closely proportional to the maximum amplitude of vibration. The values recorded by the wave analyzer are thus equal to the total vibration of the core leg and when analyzed with respect to the length of the core member, give magnetostriction values which are quite close to the values obtained on individual test strips when the apparatus of Fig. 2 is employed for measuring the magnetostriction. In measuring the vibrations, the amplifier and wave analyzer are first calibrated by measuring a known vibration so that the correct value of the vibration of the core member at any given induction can be obtained.

Referring to Fig. 7 of the drawings, there is illustrated the difference in the magnetostriction obtained with two core members of the same size constructed from the same commercially produced silicon-iron strips which have been subjected to different treatments. Curve 100 represents the magnetostriction measured on a core member of the commercially produced strips which have been subjected to only the further anneal at a temperature of 700° C., while curve 102 represents the magnetostriction measured at different flux densities for a core member of identical size formed of identical silicon-iron strip material but which has been subjected to an annealing treatment in air at a temperature of 700° C. while under a tension of 1200 pounds per square inch, and thereafter cooled under tension to approximately 100° C. The curve 100 and 102 clearly illustrate that the method of this invention when applied to commercially produced silicon-iron alloys which have been fabricated into strip form and treated to develop their magnetic characteristics is effective for reducing the magnetostriction of core members formed from the treated alloy strip.

The method of this invention is also effective in reducing the losses in core members constructed from the commercially produced alloy sheets or strips as illustrated by Fig. 6 of the drawings. In this figure, curve 104 represents the true watts loss obtained at different flux densities for the core member upon which the magnetostriction curve 100 of Fig. 7 is obtained while curve 106 represents the true watts loss at different flux densities for the core member treated in accordance with this invention and upon which curve 102 of Fig. 7 is based.

While it is not known exactly what happens in the alloy when it is treated in accordance with the method of this invention, it is quite apparent that the combination of annealing in air at a temperature within the preferred range while maintaining the strip under tension and retaining the tension on the strip until it is cooled to a temperature of about 100° C. so changes or sets the components of the alloy as to effectively reduce the magnetostriction and insure the maintenance of the reduction of the magneto-

striction at the operating temperatures of the magnetic material.

Although this invention has been described with reference to a particular embodiment thereof, it is, of course, not to be limited thereto except by the scope of the appended claims.

I claim as my invention:

1. In the method of reducing magnetostriction in a silicon-iron alloy containing up to 6% of silicon and which has been fabricated into strip form and treated to develop magnetic characteristics, the steps of, subjecting the treated alloy strip to an annealing treatment at a temperature between the Curie point of the alloy and 825° C. while applying tension to the strip, the tension applied to the strip during the anneal being below the elastic limit of the alloy strip, the tension being the only treatment applied to the alloy strip in addition to said annealing treatment for effectively reducing the magnetostriction of the alloy strip.

2. In the method of reducing magnetostriction in a silicon-iron alloy containing up to 6% of silicon and which has been fabricated into strip form and treated to develop its magnetic characteristics, the steps of subjecting the treated alloy strip to an annealing treatment at a temperature between 700° C. and 825° C. in air, while applying tension to the strip, the tension applied to the strip during the air anneal being below the elastic limit of the alloy strip, the tension being the only treatment applied to the alloy strip in addition to said annealing treatment for effectively reducing the magnetostriction of the alloy strip.

3. In the method of reducing magnetostriction in a silicon-iron alloy containing up to 6% of silicon and which has been fabricated into strip form and treated to develop its magnetic characteristics, the steps of subjecting the treated alloy strip to an annealing treatment at a temperature between 700° C. and 825° C. while applying a tension of between 500 and 2000 pounds per square inch to the strip, the tension being the only treatment applied to the alloy strip in addition to the annealing treatment, the tension applied cooperating with the anneal to effectively reduce the magnetostriction of the alloy strip.

4. In the method of reducing magnetostriction in a silicon-iron alloy containing up to 6% of silicon and which has been fabricated into strip form and treated to develop its magnetic characteristics, the steps of, subjecting the treated alloy strip to an annealing treatment at a temperature between 700° C. and 825° C. in air, while applying a tension of between 500 and 2000 pounds per square inch to the strip, the tension being the only treatment applied to the alloy strip in addition to the annealing treatment, the tension applied cooperating with the anneal to effectively reduce the magnetostriction of the alloy strip.

5. In the method of reducing magnetostriction in a silicon-iron alloy containing up to 6% of silicon and which has been fabricated into strip form and treated to develop the magnetic characteristics, the steps of passing the heat

treated alloy strip through an annealing chamber, subjecting the alloy strip to a temperature between 700° C. and 825° C. in the annealing chamber while applying tension to the strip as it passes through the annealing chamber, the tension applied being below the elastic limit of the alloy strip, and cooling the heated alloy strip under tension from the annealing temperature to a temperature of about 100° C., the tension being the only treatment applied to the alloy strip during the heating and cooling of the strip, the tension applied cooperating with the heating and cooling treatment to effectively reduce the magnetostriction of the alloy strip.

6. In the method of reducing magnetostriction in a silicon-iron alloy containing up to 6% of silicon and which has been fabricated into strip form and treated to develop the magnetic characteristics, the steps of passing the heat treated alloy strip through an annealing chamber having open ends, subjecting the alloy strip to a temperature between 700° C. and 825° C. in the annealing chamber in air while applying tension to the strip, the tension applied being below the elastic limit of the alloy strip, and cooling the heated alloy strip in air under tension from the annealing temperature to a temperature of about 100° C., the tension being the only treatment applied to the alloy strip during the heating and cooling of the strip, the tension applied cooperating with the air heating and cooling treatment to effectively reduce the magnetostriction of the alloy strip.

7. In the method of reducing magnetostriction in a silicon-iron alloy containing up to 6% of silicon and which has been fabricated into strip form and treated to develop the magnetic characteristics, the steps of passing the heat treated alloy strip through an annealing chamber, subjecting the alloy strip to a temperature between 700° C. and 825° C. in the annealing chamber while applying a tension of between 500 and 2000 pounds per square inch to the strip, and cooling the heated alloy strip under tension from the annealing temperature, the tension being the only treatment applied to the alloy strip during the heating and cooling of the strip, the tension applied cooperating with the heating and cooling treatment to effectively reduce the magnetostriction of the alloy strip.

8. In the method of reducing magnetostriction in a silicon-iron alloy containing up to 6% of silicon and which has been fabricated into strip form and treated to develop the magnetic characteristics, the steps of, passing the heat treated alloy strip through an annealing chamber having open ends, subjecting the alloy strip to an annealing treatment at a temperature between 700° C. and 825° C. in the annealing chamber in air while applying a tension of between 500 and 2000 pounds per square inch to the strip for a period of time of from one to two minutes, the tension being the only treatment applied to the alloy strip in addition to the annealing treatment, the tension applied cooperating with the anneal to effectively reduce the magnetostriction of the alloy strip.

STEPHEN L. BURGWIN.